

Aug. 4, 1942.

H. G. HALL ET AL

2,291,961

METHOD OF INSULATING ELECTRICAL CONDUCTORS

Filed March 18, 1939

2 Sheets-Sheet 1

*Fig. 1.*



*Fig. 1.*



HARRY G. HALL  
LASZLO I. KOMIVES  
INVENTORS

BY *Cleveland B. Hellebaugh*

ATTORNEY

Aug. 4, 1942.

H. G. HALL ET AL

2,291,961

METHOD OF INSULATING ELECTRICAL CONDUCTORS

Filed March 18, 1939

2 Sheets-Sheet 2



FIG. 2



FIG. 3

ATTORNEY

## UNITED STATES PATENT OFFICE

2,291,961

## METHOD OF INSULATING ELECTRICAL CONDUCTORS

Harry G. Hall and Laszlo I. Komives, Detroit,  
Mich., assignors, by mesne assignments, to  
Hercules Powder Company, Wilmington, Del.,  
a corporation of Delaware

Application March 18, 1939, Serial No. 262,614

3 Claims. (Cl. 174—19)

This invention relates to a method of insulating an electrical conductor and more particularly to a method of insulating high tension cable conductors at points where the conductors are joined or where they are terminated in order to attach them to switches and other apparatus.

The prior art has always experienced some difficulty with migration of the oil, with which the paper insulation on the cables has been impregnated, in the early installations where low potentials were utilized. This proved to be troublesome but was considered to be more or less a nuisance and not worth spending money to eliminate. However, as the art has gone to higher and higher potentials and the viscosity of the impregnating compounds has been constantly decreased in order to obtain lower dielectric losses, the frequency of oil migration increased and within the past 10 years or so has become a critical factor in cable installations. It has been especially true on high tension cable systems, where so-called hard filling compounds, have been used on cable accessories such as joints, terminals, etc.

Prior art filling compounds when used in cable joints, for example, have all had a tendency to dissolve in the oils with which the paper insulation used on cables has been impregnated. This oil solubility has resulted in innumerable failures on the high tension cable lines because of swollen, collapsed or burst joint sleeves. Solution of the joint-filling compound in the cable oil has materially increased the power factor and dielectric loss of the cable to a point where failures have occurred in the cable due to heating of insulation, because of migration of the dissolved filling compound into the cable. Furthermore, once a compound is dissolved in the joint, a channel may exist thru the joint which may allow oil to drain from the cable at higher points and thus cause cable failure because of imperfectly impregnated cable at such locations.

The trouble with oil migration from terminal boxes into the cables has also become critical during the last few years, especially with high tension installations. High power factor and dielectric loss may result when oils of different characteristics are mixed. Numerous ways have been devised for obviating this difficulty but none have resulted in more than temporarily checking the flow of oil. It has long been known that mineral oil is a superior filling material for cable terminals, provided that some method could be devised to prevent the mineral oil in the cable terminal from soaking into the insulation of the

cable and thus displacing the heavier oils with which the paper insulation is impregnated to the detriment of both the cable and the terminal.

It is an object of this invention to provide a method whereby joint failures, due to the oil solubility of the insulating compound used in making the joint, are substantially completely obviated.

It is a further object of this invention to provide a means for preventing the migration of mineral oil from cable terminals into the paper insulation of the cable.

Further objects of this invention will appear hereinafter.

These objects are accomplished by the following invention which consists broadly of providing a method of insulating electrical conductors by surrounding said electrical conductors with a hollow body and substantially filling the space intervening between the conductors and walls of said hollow body for at least a portion of the total length of said hollow body, with an insulating composition comprising a mixture of a natural glyceride and petroleum hydrocarbon-insoluble resin derived from pine wood.

Having now indicated in a general way the nature and purpose of this invention, there follows a more detailed description of the preferred embodiments thereof with reference to the accompanying drawings in which:

Figure 1 represents a view of a cable joint, partly in cross section.

Figures 2 and 3 show the method of using the insulating compound in accordance with this invention for insulating electrical conductors in a cable terminal box.

Figure 4 represents an alternative method which may be used for insulated electrical conductors in a cable terminal box. The method here shown, however, is limited to insulations in a cable terminal which is in a vertical position.

Referring now particularly to Figure 1 the ends of lead-sheathed cable 1 to be joined, are opened, and the lead sheathing removed therefrom for a distance back to the end of each to allow suitable manipulation. Various layers of oil-impregnated paper insulation 2 are removed from the conductors, laying bare the cable conductors 3. The cable conductors 3 are so arranged that the ends of the bare copper are held squarely together by a soft copper sleeve 4 of a diameter somewhat more than the conductor 3 and of sufficient length to extend far enough over the joint to make substantial mechanical and electrical contact. The ends of sleeve 4 are filed

so as not to leave any sharp edges, then carefully hammered down in order to fit snugly, filed smooth and then sleeve 4 is soldered to conductors 3.

After the conductors have been joined, a lead sleeve 5 of a large section with respect to the lead sheathed cable and of sufficient length so that the ends thereof extend appreciably beyond the point where the cables have been opened, is then placed over the joint. Lead sleeve 5 is fastened to the lead sheathed cable 1 by applying a wiped solder joint 6 to each end of sleeve 5. Lead sleeve 5 is then filled with a hot composition 7 at a temperature sufficiently high to have the resin present in a molten state, comprising a natural glyceride and petroleum hydrocarbon-insoluble resin derived from pine wood, and after cooling of this insulating composition, sleeve 5 is sealed, by soldering, or in any other manner well known to the art.

This invention relates particularly to a method of insulating conductors in a cable terminal box. The embodiment shown in Figures 2 and 3 is especially adapted for use where the end of the cable enters the cable terminal box horizontally. Referring particularly to Figure 2, lead sheathed, paper insulated, multi-conductor cable 10 is inserted horizontally thru one side of cable terminal box 12, only a portion thereof being shown, said cable 10 being fastened to cable terminal box 12 in the manner shown or in any other manner well known to the art. Lead sheathing is then removed from a portion of cable 10 which projects into cable terminal box 12, exposing the paper insulated conductors 13, for a distance depending on the voltage at which cable 10 is to operate. The paper insulated conductors 13 are then wrapped with an insulating tape 14 which is coated or impregnated with an insulating composition comprising a natural glyceride and petroleum hydrocarbon-insoluble resin derived from pine wood taking particular care to cover all of the exposed paper insulation on the conductors. In most cases, it will be desirable to have a multiplicity of layers of tape. A flexible glove 15 made of rubber or of similar material capable of being readily shaped to conform to the spaced arrangement of the conductors is then placed over conductors 13 leaving a thumb 16 of glove 15 free. The fingers of glove 15 are open at the end and the ends of the fingers engaging the insulated conductors 13 are then wrapped with cord to form a tight joint with the insulation. The wrist of glove 15 is similarly wound to the lead sheath of cable 10.

A hot composition 17 at a temperature sufficiently high to have the resin present in a molten state, comprising a natural glyceride and petroleum hydrocarbon-insoluble resin derived from pine wood is then poured in through thumb 16 filling the glove with said composition. After the composition 17 has cooled, thumb 16 of glove 15 is folded down and tied as shown in Figure 3 and then several layers of tape coated or impregnated with insulating composition 17 applied about the glove 15. Cable terminal box 12 is then filled with an insulating oil, for example, a suitable mineral oil. Because of the insolubility of our insulating composition in mineral oil, a complete stop is provided which prevents the mineral oil from entering the paper insulation of cable 10.

Although, as stated before the method above described is particularly applicable for use where the cable enters the box horizontally, it is also

applicable where the cable terminal box is vertical, shown in Fig. 4, especially if the horizontal surface inside the box 28 is extensive. If this surface can be made relatively small, however, an effective oil stop may be made in a somewhat simpler manner, referring particularly to Figure 4. Lead sheathed cable 10 is brought into the bottom of the cable terminal box 28 in a manner similar to that in which it is brought in the side of the box as shown in Figures 2 and 3. The lead sheathing on cable 10 is then removed, exposing the paper insulated conductors for a distance depending on the voltage at which the cable is to operate. These paper insulated conductors are then wrapped with multiple layers of tape 14 coated or saturated with a composition comprising a natural glyceride and petroleum hydrocarbon-insoluble resin derived from pine wood completely covering all exposed paper insulation. A hot composition 17, at a temperature sufficiently high to have the resin present in a molten condition, comprising a natural glyceride and petroleum hydrocarbon-insoluble resin derived from pine wood is then poured into the bottom of cable terminal box 28 in amount sufficient to cover all of lead-sheathed cable 10 projecting through the bottom of cable terminal box 28 and a small portion of the insulated conductors 13, wrapped as shown above. After the insulating composition 17 has cooled and is a solid mass, the balance of cable terminal box 28 is then filled with a suitable insulating composition such as, for example, a suitable mineral oil. Since our insulating composition, which is at the bottom of cable terminal box 28, is insoluble in oil, an effective stop is provided to the migration of oil into the cable.

The petroleum hydrocarbon-insoluble resin derived from pine wood may be prepared by extracting pine wood with a coal tar hydrocarbon such as benzol or toluol, then evaporating the volatile constituents leaving a residue consisting of a mixture of wood rosin and the resin used in the present invention. Extraction of this mixture with a petroleum hydrocarbon such as, for example, gasoline, dissolves the rosin, and after separation of the rosin high in abietic acid, there remains a resinous residue, low in abietic acid. This resinous residue is characterized by substantial insolubility in cold petroleum hydrocarbons but will differ somewhat in its specific characteristics such as acid number, melting point, exact petroleum ether solubility, and content of naphtha and toluol soluble matter depending upon the method of the recovery of rosin from pine wood used in its production. Where, in the specification and claims, we refer to petroleum hydrocarbon-insoluble resin derived from pine wood, we mean that said resin is substantially insoluble in petroleum hydrocarbons such as, for example, gasoline, petroleum ether, hexane, heptane or operable equivalents.

The natural glyceride may be an animal or vegetable oil as, for example, castor oil, polymerized castor oil, soya bean oil, cotton seed oil, China-wood oil, cocoanut oil, perilla oil, olive oil, linseed oil, etc., and may be admixed with the petroleum hydrocarbon-insoluble resin derived from pine wood in widely varying amounts for the purpose of the present invention. We have found that a range from about 1% to about 70% oil, the balance being resin, is satisfactory depending upon the particular characteristics desired in the combined insulating compound. For

most purposes, however, we prefer to use from about 10% to about 60% oil in our compositions.

We have found that a mixture comprising 70% petroleum hydrocarbon-insoluble resin derived from pine wood and 30% castor oil is particularly effective as an insulating compound for use in accordance with the present invention. While any natural glyceride may be used, the use of castor oil, either raw, blown or polymerized is preferred, as this compound is most resistant for long periods to the action of petroleum hydrocarbons such as will be present in mineral oils and in impregnated paper insulated cables.

Although any procedure may be used to combine the resin and oil, we prefer to combine and blend the oil and the petroleum hydrocarbon-insoluble resin derived from pine wood by fusing this resin at a temperature slightly above its melting point and then adding and thoroughly admixing with this fused resin the desired amount of the oil. After mixing, the mixture may be allowed to cool and may be used from time to time merely by reheating to the point where the combination is fluid. For the purposes of the present invention, we prefer to have the compound at a temperature of approximately 250° F. when pouring the composition into the flexible glove or into the lead sleeve.

In order to show the particular effectiveness of the insulating compositions made in accordance with the present invention, the following data are shown. Four compounds were made, varying the amount of petroleum hydrocarbon-insoluble pine wood resin in each case. The oil-resin mixtures were prepared by adding the resin to the oil gradually. During the mixing, which required from 2 to 4 hours, the mixtures were kept at a temperature of 100° C. to 130° C. and were mechanically stirred. These mixtures, to which we shall hereinafter refer as A, B, C, and D had the following composition in per cent by weight.

| Mixture | Per cent petroleum hydrocarbon-insoluble pine wood resin | Per cent castor oil (cold pressed) |
|---------|----------------------------------------------------------|------------------------------------|
| A       | 85                                                       | 15                                 |
| B       | 70                                                       | 30                                 |
| C       | 60                                                       | 40                                 |
| D       | 33                                                       | 67                                 |

A small weighed crucible filled with each of these compounds was then immersed in individual flasks containing 150 ml. of unused insulating oil. These flasks together with the crucibles were kept in an oven at 65° C. for one week after which the crucibles were removed, wiped free from oil with a dry cloth, and reweighed, the loss in weight measuring the solubility of the compounds in the oil. A power factor test was then made on the oil to determine the extent of damage to the oil by the material dissolved therein.

Brittleness point of the mixtures was determined by filling the space between a single conductor, including paper tape, and a section of a lead cable sheath,  $\frac{1}{2}$  inch by  $2\frac{3}{4}$  inches, with the mixtures under consideration. The specimens so prepared were slowly cooled from room temperature to 0° F., the compounds being visually examined for cracks and surface checking at each 10° F. interval. The temperature at which cracking occurred was taken as the brittleness point.

The data obtained are shown in the following table:

TABLE I

| 5                                                             | Compound | A       | B       | C       | D |
|---------------------------------------------------------------|----------|---------|---------|---------|---|
| Brittleness point.....°F.                                     | 10-20    | Below 0 | Below 0 | Below 0 |   |
| Solubility in oil at 65° C.<br>Loss in wt. of cpd<br>per cent | 0.06     | 0.31    | 0.91    | (*)     |   |
| 10 Power factor of oil after<br>immersion of cpd.**           | 0.0030   | 0.0018  | 0.0013  | 0.0030  |   |
| Power factor of oil before<br>immersion.....                  |          | 0.0014  |         |         |   |

\*Not determined—too fluid.

\*\*Power factor measured at 80° C. at a voltage stress of 50 volts per mil.

The above table clearly shows the insolubility of the insulating compositions, used in accordance with the present invention, in an electrical insulating oil. The power factor of the oil, after test, indicates that no material damage has been done to the oil. In fact the maximum difference of 0.0016 from the value of 0.0014 for the new oil, can be considered to be so small as to be negligible for all practical purposes. Solubility of prior art joint filling compositions in the insulating oil caused the power factor of the oil to increase enormously and this has been one of the most serious disadvantages of prior art compounds. This disadvantage is, however, completely overcome by the present joint filling compounds.

In the following table, the effect on the power factor of an insulating oil is shown, by the addition thereto of minor amounts of a joint filling compound. The power factor measurements, as in the previous table, were made at a voltage stress of 50 volts per mil.

TABLE II

| 40 | Percent compound in insulating oil                     | Power factor |        |        |        |
|----|--------------------------------------------------------|--------------|--------|--------|--------|
|    |                                                        | 20° C.       | 40° C. | 60° C. | 80° C. |
| 45 | Insulating oil alone.....                              | 0.0002       | 0.0004 | 0.0012 | 0.0024 |
|    | 0.5% mixture B.....                                    | 0.0004       | 0.0011 | 0.0051 | 0.0098 |
|    | 0.5% asphaltic cpd.**                                  | 0.1214       | 0.2790 | 0.5012 | 0.7217 |
|    | 1.0% of 1:1 cable impregnating cpd. and mixture B..... | 0.0001       | 0.0002 | 0.0007 | 0.0021 |

\*Compound completely soluble in the oil.

50 The remarkable superiority of the joint filling compounds used in the present invention over prior art compounds is clearly indicated by the above table. The petroleum hydrocarbon-insoluble pine wood resin—glyceride oil compositions of the present invention are so insoluble in the electrical insulating oil that their presence has no deleterious effects on the electrical characteristics of these oils.

In the following Tables III and IV, various 60 electrical characteristics are given of the compositions formulated as before shown.

TABLE III  
Dielectric strength of mixtures A, B, C, and D  
(A. S. T. M.—D176—36T)

| 65 | Mixture | Breakdown voltage kilovolts 0.05 inch gap |        |        | Dielectric strength volts per mil |        |        |
|----|---------|-------------------------------------------|--------|--------|-----------------------------------|--------|--------|
|    |         | 30° C.                                    | 60° C. | 90° C. | 30° C.                            | 60° C. | 90° C. |
| 70 | A       | 65.2                                      | 42.8   | 26.5   | 1,304                             | 856    | 530    |
|    | B       | 41.5                                      | 29.3   | 22.2   | 930                               | 586    | 444    |
|    | C       | 28.5                                      | 22.3   | 18.5   | 570                               | 446    | 370    |
| 75 | D       | 22.8                                      | 21.2   | 12.5   | 456                               | 424    | 250    |

TABLE IV  
Power factor of mixtures A, B, C, and D (measured at 60 cycles and voltage stress of 2.32 volts per mil)

| Mixture | Power factor |        |        |
|---------|--------------|--------|--------|
|         | 30° C.       | 60° C. | 90° C. |
| A.....  | 0.0594       | 0.1049 | 0.1460 |
| B.....  | 0.0640       | 0.0833 | 0.1234 |
| C.....  | 0.0677       | 0.2056 | 0.9680 |
| D.....  | 0.1308       | 0.8829 | 0.9550 |

The method of insulating electrical conductors through the use of an insulating composition, comprising a natural glyceride and substantially petroleum hydrocarbon-insoluble resin derived from pine wood in accordance with the methods before described has proved to be eminently satisfactory in practice. In the case of cable joints, our insulating compound possesses the insulating and other electrical characteristics necessary to insulate high tension conductors one from the other in the case of multiple conductor cables and the conductor or conductors from the grounded lead sheath of the cable or the lead sleeve of the cable joint, without the expensive application of insulating tape over the conductors at the joint, which has been essential in all of the prior art cable joints.

Furthermore, as the data before show, the petroleum hydrocarbon-insoluble pine wood resin-glyceride oil combinations, because of their insolubility in the oils commonly used in electrical work, make possible a joint which has for all practical purposes an indefinite life. On the other hand, prior art joint filling compounds were all more or less miscible with the cable oils. As these materials mixed, the power factor increased with a consequent rise in temperature producing ultimately a cable failure. By preparing joints in accordance with the present invention the possibility of joint failure is practically eliminated.

While it is possible by prior art methods to prevent oil from entering the conductor insulation on a three conductor cable, for example, in a cable terminal installation, for a period of time, there is no assurance that the installation will remain tight during the life of the equipment. This, as the data before clearly show, has been accomplished by utilizing methods in accordance with this invention.

In connection with cable terminal installations, the oil tightness of the open cable cross-section other than the conductor insulation itself is an even more difficult undertaking because of the uneven configurations which have to be taken into account. Due to repeated cooling and heating of the line, the relative position of the three conductors at the end of the cable changed quite considerably and caused holes to be formed in prior art tapings which to outside appearances and even under tests, appeared to be oil tight. To compensate for this movement, it is necessary to have the sleeve or taping around the conductors surrounded by a plastic compound held in position with an elastic ma-

terial. This is successfully accomplished by the method in accordance with our invention because our insulating composition remains plastic at all operating temperatures and it is surrounded by a flexible glove which is elastic and in itself oil resistant.

It will be understood that where we refer to an electrical conductor, we mean either a single conductor or multiple conductors.

10 It will be further understood that the details given hereinbefore are illustrative only and in no way limiting on our invention as broadly described hereinbefore and in the appended claims.

What we claim and desire to protect by Letters Patent is:

1. A method of terminating an electrical cable in a cable terminal box, said cable comprising a plurality of conductors each of which is insulated with an oil-permeable insulation, which comprises fitting the cable receiving portion of a flexible casing around said cable and fitting the conductor receiving portions of said casing around said insulated conductors, filling said casing with a fluid oil-resistant insulating composition comprising a mixture of a natural glyceride and a petroleum hydrocarbon insoluble resin derived from pine wood, wrapping said casing with servings impregnated with said insulated composition, and filling the cable terminal box with an insulating oil.

2. In a cable terminal structure, the combination of a cable comprising a plurality of conductors each of which is insulated with an oil-permeable insulation, a flexible casing including a pour opening and a plurality of tubular conductor receiving portions and a tubular cable receiving portion receiving said cable and conductors in such manner that the cable receiving portion of said casing receives a portion of said cable and the conductor receiving portions receive a portion of the conductors, an oil-resistant insulating composition comprising a mixture of a natural glyceride and a petroleum hydrocarbon insoluble resin derived from pine wood filling the space between said casing and said cable and conductors, a terminal box enclosing said casing, and an insulating oil filling the space between said casing and said terminal box.

3. A method of sealing the insulating material of an electrical cable against migration loss, said cable comprising a plurality of conductors spreading from one end of said cable and being insulated with an oil impregnated dielectric material, which comprises fitting a flexible casing including a pour opening, a cable receiving portion and a plurality of conductor receiving portions around said conductors, securing the terminal ends of said portions in close fitting relationship to said conductors and said cable end, filling said casing through said pour opening with a molten composition comprising a mixture of a natural glyceride and a petroleum hydrocarbon insoluble resin derived from pine wood, and allowing said mixture to solidify, whereby the oil of said material is sealed and held in insulating position.

HARRY G. HALL.  
LASZLO I. KOMIVES.